

# UNITED STATES PATENT OFFICE.

ANDREW THOMA, OF CAMBRIDGE, MASSACHUSETTS, ASSIGNOR TO NORTH AMERICAN CHEMICAL COMPANY, OF BOSTON, MASSACHUSETTS, A CORPORATION OF MAINE.

## SHOE-BOTTOM FILLER.

1,134,931.

Specification of Letters Patent.

Patented Apr. 6, 1915.

No Drawing.

Application filed November 7, 1910. Serial No. 591,207.

To all whom it may concern:

Be it known that I, ANDREW THOMA, a citizen of the United States, residing at Cambridge, in the county of Middlesex and 5 State of Massachusetts, have invented an Improvement in Shoe-Bottom Fillers.

Practical experience with my commercial shoe bottom fillers has made evident to me that one of the prime essentials of a granular filler material is that it shall not merely contain components whereby the ground cork and binding agents may be readily mixed together, but shall contain components which shall cause the said mixture to 10 remain unchanged for a sufficient length of time to allow its proper installation within shoe bottoms (in accordance with the usual relatively long delays common in shoe factories). Therefore, according to my present 15 invention, the shoe filler is not only sticky and possessed of the general properties set forth in my Patent No. 945,294 of Jan. 4, 1910, but when set to a certain degree it is thereafter slow hardening. By this I mean 20 that it is quick setting to that consistency which is requisite for the filler lodged in the shoe bottom while awaiting the sole laying process, but, having thus quickly set to said 25 consistency or condition of stiff plasticity, the further setting or hardening comes then 30 practically to a halt, so that from that point forward the preparation is characterized by being slow hardening and slow drying. A further characteristic is that the filler does 35 not dry out (in the way, for instance, as would be expected of a gluey or gelatinous compound, in accordance with the nature or commonly recognized properties of glue or gelatin), but for days remains tacky or 40 sticky, like ordinary rubber-cement filler. A third important feature of the invention is that the filler remains yielding and conformable during the sole laying operation under the "leveling process" to which the 45 shoe bottoms are subjected during the manufacture of the shoes and yet later becomes tough and substantially non-conformable, without however becoming dry, hard, stiff or unyielding. The leveling pressure requires 50 that the filler material shall remain conformable so as not to interfere with the proper shaping of the shoe bottom, and yet shall remain sufficiently sticky, adhesive and cohesive so as not to be materially influenced 55 by the crowding pressure of the leveling machine, and accordingly it is one object of my invention to attain this result in a superior degree (the process or method, broadly considered, being duly claimed in my copending 60 application Serial No. 687,385, now Patent No. 1,036,931, dated August 27, 1912). This point will be clearer by bearing in mind the contrast of my filler, although preferably containing glue or glue-like components, over the natural characteristics of glue, 65 which, when set, does not allow itself to be disturbed without loss of cohesion and adhesion. Furthermore, my present filler, although it does not attain its permanent set condition until the shoe has been completed, 70 is then not only tough but is also firm holding so as to retain tenaciously its grip against the leather of the innersole and the outersole. Likewise it is water repellent (the large proportion of the naphthalene 75 influence being very effective), and is adapted to a commercial packaging without suffering loss of quality or usefulness through storage, and is especially suitable for subsequent spreading of the mass within shoe 80 bottoms, and stays where put, i. e., it does not slide away. When set to its permanent condition, the binding medium and ground cork form a rubber-like mass in that it is absolutely non-shifting and tough and yet is 85 yielding so as to form a proper cushion for the foot of the wearer of the shoe, but it is not "drawing" or heavy and dense.

Preferably my present invention is of the same nature as in my Patent No. 945,294 90 aforesaid, and is subordinate thereto. I have found the use of glue very useful, as stated in said patent, as a chief component of shoe bottom filler, using said term herein to include the variety of mixtures 95 suitable for said purpose as set forth in said patent, and among which may be enumerated (from said patent) albumen glue, casein glue, starch glue, vegetable glue, marine glue.

One object of my present invention is to provide specific means in the form of chemical reactions and combinations, for rendering the glue (by which term I include the various gelatinous components mentioned in 105 said patent) fluid, sweet and wholesome, and

to protect it against deterioration, precipitation or separation from its solvent or other admixed ingredients under ordinary atmospheric conditions such as are met with in general commercial use.

5 A further object of my invention is to provide a compound in which the means used for thus preserving the proteid matter is sufficiently simple, effective, inexpensive and harmless (to the leather, stitching and adjacent fabric) to render it practical for the handling of large quantities of material, as required in the commercial manufacture of shoe bottom filler.

15 When carried out in its preferred form, my invention is capable of providing a binding constituent or binding cement which may be itself stored without undergoing objectionable change, so as to be ever ready to be intermixed (as the binding medium or agent) with the granular body (preferably ground cork) of the filler material to be placed within the shoe bottoms. The cementitious portion or binding agent may 20 be admixed with the granular body in a cold state and the completed mixture or shoe bottom filler may be then applied in a cold state to the shoe bottom. This method is preferable from the standpoint of convenience as it simplifies the operation and promotes the comfort of the operator, but my 25 filler is intended also to be subservient to heat application. In the latter instance a less amount of water is required in the filler 30 and it is therefore quicker setting. As however the water solvent of my filler is less paramount or assertive than in ordinary glue solutions, it does not interfere with the drying and setting of the installed material 35 sufficiently to require the heating process. Glue is desirable as a binding medium because it possesses in itself the qualities of 40 tenacity and stickiness requisite to unite parts strongly and firmly, but it is not water repellent and when set it lacks a surface sufficiently sticky or adhesive to assist in the 45 attaching of an outersole to the prepared shoe bottom (which does not take place, in practice, until quite a while after the filler 50 is applied). On the other hand, I have found that a great many of the sticky, gummy, cement-components which might otherwise be fit to be used for shoe filler purposes, are rendered unfit by lacking the 55 aforesaid qualities of tenacity and strength which are so abundant in glue. Accordingly it is the object of my present invention to unite these different factors in such a manner as to gain the desired results,— 60 and it will be noted that said results are gained, by my invention, in a surprising degree.

The sticky adhesive of my preparation is preferably a natural product, which may 65 be sticky and workable in itself, or of an

artificial resinous nature, preferably prepared by treating resins with dissolving or fluxing means which render them soft, sticky or pitchy. Aside from these are other artificial products fit to be used for my 70 purpose, such as tarry pitches like stearin pitch and the various petroleum pitches, or similar preparations having like properties and therefore capable of forming the desired sticky element mentioned for combination with the tenacious or strong and tough glue solution mentioned. I have found, for instance, that by subjecting five parts of rosin to one part of naphthalene to a melting process, these two solids produce 80 a semi-fluid mass which is very sticky and adhesive (and which in my Patent No. 1,121,054, dated December 15, 1914, I have called a "resin naphthalate"). By melting six parts of glue in ten parts of water and adding to 85 the heated solution two parts of chlorid of calcium and five parts of the above naphthalene and rosin, I obtain a cementing fluid which is of transparent, smooth-flowing consistency, well adapted to my purpose. The 90 chlorid of calcium renders the glue fluid and stops the jellifying of the same, and thereby afterward renders the glue component of the filler slow-drying. The action of the chlorid of calcium is not only effective 95 on the glue portion of the preparation, but is equally beneficially active on the rosin paste by furthering the chemical union between the two ingredients. The dissolving action of the naphthalene on 100 the rosin is such that the latter component is in the state of a paste when admixed with the glue solution, but on account of the thorough amalgamation of the whole mixture I 105 am led to believe that the said solvent is also effective on the glue component, as the union or chemical coalescing is surprisingly thorough and perfect and without trace of separation,—this being one of the desirable objects to be attained. Aside from the fluxing 110 action of the naphthalene, its presence is most effective as a preservative and sweetener of the proteid matter, and it therefore fulfils a double purpose, especially when it is borne in mind that this filler material is 115 manufactured in large quantities in liquid form but is often stored for months before it is finally used. An addition of two parts of glycerin to the above formula gives to the filler mass when set, a greater resiliency. Olein oil is a desirable agent either with or 120 without the glycerin, for softening the mass or rendering the gluey component more flexible, as hereinafter explained at more length.

I have given the above special formula merely as an illustration to explain the general composition of my preparation, for it will be readily understood that large variations can be made without materially modi-

fying the ultimate objects and advantages of the cement. For instance, casein, starch, dextrins, mucilaginous gums, or like products, may be substituted for all or part of the glue component, thereby diffusing the toughening influence of the glue throughout a larger and cheaper mass and not only altering the proportionate amount required of the chlorid of calcium, but bringing into play other chemical ingredients which in a like manner influence the solvent parts to effect a more fluid condition. Thus, whenever it is desired to give the water-absorbent, stiffening portion of the compound an appearance of bulk, satisfactory results are obtainable by a combination of the glue as a toughening means with the fluffy starch preparations (such as apparetaine, *i. e.* starch-glue, for example), wherein the glue constitutes the tempering or toughening component for the firmer-setting starch. Again, solutions of dextrin or casein or both can be tempered in the same way by glue, thereby spreading, so to speak, the effectiveness of the glue when very plastic (for instance) throughout the mass of the much cheaper dextrin, casein, etc. This illustrates the scope and effectiveness of the toughening, water-absorbent component. The same is true of the water repellent, sticky, resinous component, (*i. e.* large variations of other ingredients may be substituted in whole or in part for this portion of the compound), as will appear more fully later on in this specification. Various combinations of resinous, tarry, or pitchy ingredients may be provided by fluxing the same to the desired consistency, with or without the dissolving influence of naphthalene. In fact, the rosin component may be added in the form of resinates, rosin soaps, or emulsions, without departing from the principle of supplying this particular element to my solution. A compound even less thoroughly amalgamated than in the specific illustration above, and formed of components averse to a complete fluxing into one another, may accomplish the purpose of uniting the granulated filler-material within the general meaning and composition of my preparation and invention, as appears later herein. The chlorid of calcium has the advantage of being very cheap, but instead thereof chlorid of magnesium may be used, or chlorid of zinc or alkalies, acids, or both, so as to neutralize one another in the preparation and thus become the means of accomplishing the chemical union or fluidifying of the ingredients. Also, although more expensive, I have found the use of alizarin or water-soluble oils effective for the modifying purpose described in connection with my preparation, the dissolving action thereof being equally effective on both glue and resinous matter. On the other hand, a considerable variety of oils can

be used to act as a softening agent on the resins alone or on both of the principal components of the cementitious liquid.

The formula thus far discussed has been chosen for that purpose as being the best with which to explain, not only the components required, but also their relation to, and action on, one another, and especially the novelty of the combination and its consequent results. I have endeavored by this formula to present a clear, concise illustration of the principles and objects or results of my invention, which latter has a wide scope of composition, use, and advantages. In this illustration, the slow-drying principle sought for is controlled by the action of the chlorid of calcium upon the proteid matter and by the naphthalene in its dissolving and slow-evaporating union with the resin, but many substitutes may be used for these ingredients. The glue would normally tend first to jellify (in connection with water) and then, when applied, would keep on hardening until it got brittle (in its original state). This is prevented for the time being by the chlorid of calcium, so that it is slow in tending to get to this point. The glycerin gives the glue resiliency and pliability or softness. The product of rosin and naphthalene introduces the sticky element in such form as to be equally slow drying and works in harmony with the gluey component and coalesces perfectly with the same on account of the presence of the chlorid of calcium. The olein oil, virtually a chemically treated castor oil, enters in complete union with both the gluey and the resinous components on account of its peculiar solubility, *i. e.* it fluxes with water on the one hand and oil on the other hand in a remarkably practical manner. I aim to render the glues soluble and liquid in such a manner as decidedly to modify their tendency to harden or gelatinize (or jellify) without impairing their tenacity or strong adhesiveness, so that they will tend to remain for a long time relatively clear and syrupy, and this tenacious syrupy component is so combined with the normally sticky, tacky resinous component that the short, weak adhesiveness of the latter is eliminated from the compound, or rather is strengthened into a tough cohesion and adhesion, while the non-sticky and non-tacky, brittle or non-shiftable normal (*i. e.* when set) quality of the gluey component is eliminated or changed into a sticky tractable or modable and impressible component, which, when the compound is mixed with the ground cork (or other filler base), will retain its laid shape, but not rigidly so, being responsive to pressure, *i. e.*, being somewhat elastic or tending to resume its original shape when momentarily distorted. When the ingredients are brought together so as to combine these two primary principles,

and in accordance with the foregoing explanation, the filler is quicksetting in the sense of stiffening at once upon being spread out thin in the shoe-bottom, but without becoming hard or dry, and thereafter it is extremely slow hardening or drying, and has the further characteristic of always holding tenaciously together in a permanently moldable or conformable and elastic body.

10 In further explanation of the wide range of chemical components contemplated, it may be pointed out that, without making any change in the before explained tenacity-giving component of the solution, namely 15 the glue, I have found that as a substitute for the six ounces of the product of naphthalene and rosin of the before-mentioned formula, I can use, for instance, five ounces of white pine pitch (a semi-soft sticky 20 exudant from certain pine trees), and from one half to one ounce of naphthalene (according to the consistency of the white pine pitch), or I can use five ounces of fir balsam (a sticky vegetable product similar to 25 the white pine pitch) and the same one half to one ounce of naphthalene, or six ounces of crude turpentine (sometimes called Venetian turpentine), or five ounces of Burgundy pitch and one to one and one half 30 ounces of naphthalene (when the pitch is semi-soft, but when harder a large proportion of naphthalene is required). Instead of the naphthalene, I may use another slow-drying solvent for the sticky resinous 35 component, such, for instance, as creosote extract, which is very practical for my purpose in rendering the resin sticky and adhesive. In like manner, pure tar, often called Stockholm or Wilmington tar, can be used 40 to accomplish the reduction of the resins to the desired sticky, semi-soft condition. On account of the natural variation of the different creosote liquids (which range from a water white to thick dark fluids), it is 45 somewhat difficult to give accurate proportions, so that the best I can do is to state a formula which gives the right proportion for the creosote of a specific gravity test (from which any one skilled in the art can 50 determine the right proportion of any other range of creosote) as follows: six parts glue in ten parts water, two parts chlorid of calcium, two parts glycerin, five ounces white pine pitch, and two ounces creosote of a specific 55 gravity of 0.980. Or, for the sticky resinous component, I may use thin fir balsam, or may use rosin, or Burgundy pitch. On account of the dark brown nature of the Wilmington pine tar, which is still more increased through concentration by the heat, 60 the resulting liquid binder of the filler when made therewith is of a darker nature and hence somewhat objectionable on this account, besides its strong peculiar tarry odor, 65 but is otherwise capable of producing, in combination with resins, a very serviceable sticky mass, two parts of the pine tar being used to five parts of rosin, etc. In fact, Stockholm tar can be reduced by boiling to a plastic condition as described without any 70 additional resinous ingredients. I may also class among these dark ingredients, stearin pitch, which often is sold to the trade in the desired soft condition, but when too hard can be adjusted by solvng ingredients 75 such as previously mentioned. I wish to emphasize that the preferred method of reducing or producing these sticky components is by the use of a slowly evaporating dissolving agent whereby the drying-out of 80 the latter leaves the filler mass in a condition subservient to or responsive to the ultimate tougher conditions of the gluey or gelatinous component. On the other hand, combinations can be formed between pitches 85 and resins which bring about this slower setting of the cement binder by means of saponifying the vegetable resins similar to a soap, so that the resulting resins, in union with the glue or like bodies, produce a good 90 binding agent for the granulated cork or comminuted filler base. I have also found that alizarin oil (and the so-called soluble oil), used principally in the sizing and finishing of cloths, is capable of forming a 95 union between the glue and the resinous sticky matter, which is of special value in supplying elasticity to the glue and becoming the medium of perfect fluxing for the various components. For instance, the following formula gives good results: six parts 100 of glue in nine parts of water and two parts chlorid, four parts of alizarin oil (olein oil), and six parts of rosin. Another formula is four parts of glue in four parts of water, one and one-third part of chlorid, 105 four parts of alizarin oil (olein oil), three parts of the naphthalate of rosin, as mentioned, (i. e. the explained product of rosin and naphthalene,) six parts of plain rosin, 110 and two parts of thick viscous linseed oil. In this formula, instead of the six parts of glue of the preceding formula, I have substituted for two of said six parts of the 115 gluey tenacious matter, an equal portion (two parts) of thick, viscous linseed oil, so that the resulting preparation, although somewhat less tenacious, is in a greater degree water repellent. This latter feature can be still more improved by a larger proportion 120 of the linseed oil. The complete fluxing of these ingredients (in this last mentioned formula) results in a smooth-flowing preparation, the thickness of which is principally controlled by a proper amount of water. 125 Regarding the fluidity of the preparations in which I have included olein oil as a fluxing medium, I do not intend to limit myself to the use of water alone, as naphtha can take the place of water without any great 130

change in the ingredients and proportions, as for instance four parts of glue, five parts of alizarin oil, two parts of thick viscous oil (linseed), three parts of the naphthalene-  
5 and-rosin, and six parts of plain rosin, together with naphtha sufficient to produce the required fluidity. With water for the fluid agent, the preparation is of a creamy-white  
10 syrupy nature (*i. e.* it is what I call an emulsion, in which the resinous ingredients are saponified), while the above naphtha-solvent formula produces a rich amber color, but when the cement binder has set, the appearance of the material is the same in both  
15 uses.

I wish to emphasize the large variation of ingredients which it is possible to bring into use without departing from the spirit and scope of my invention. For instance,  
20 the formulas given to illustrate the use of alizarin or olein oil show the adaptability of this artificial water-oil in forming the medium for introducing sticky oily ingredients while still providing a thorough fluxing of the preparation. So, in some instances, it may be desirable to introduce various other gluey constituents or mucilaginous substances such as starch or starch dextrins or artificial gums made therefrom, or similar mucilaginous substances such as natural gums, gum arabic, etc. either in place of part of the previously described gluey component or of the sticky resinous ingredient or of all of the said previously described  
25 gluey components (as will appear more fully later herein). The fluxing and introduction of these starches or gums is greatly facilitated by the soluble oil. Both the olein oil and glycerin are water-soluble fat-  
30 derived oily liquids (as mentioned in my application, Serial No. 550,802, filed March 21, 1910, certain species of which application are generically claimed herein), and these oils soften and render tenacious the gummy or gluey ingredient (which includes the permanently jellified starch, already mentioned as an artificial gum or starch-glue). Said oil supplies a certain amount of softening plasticity to the set compound, is slow-  
35 drying and, on account of its peculiar solubility, forms a ready means of combining a vast variety of binding ingredients, such as proteids, caseins, starches, gums (arabic, for instance), rubber, gutta percha (and other gums cut by naphtha),  
40 oils, fats, fatty acids, resins, pitches, etc., (as mentioned also in my patent aforesaid. For instance, the aqueous soluble proteid, previously dissolved in glycerin and olein oil, as is mentioned, is united with sticky gummy materials but so as to have the water solvent sufficiently evaporated to provide for the subsequent solution thereof in naphtha and then admixed  
45 with naphtha-soluble sticky matter, such as

50 gum, rubber, gutta percha, etc., the whole, in the form of a naphtha solution, being added with the comminuted filler material to the consistency requisite for a shoe-bottom filler, *viz.* to the condition of a semi-solid self-sustaining mass. Such compounds can be used cold or hot as may be desired. To sum up, therefore, my filler, as thus far discussed, would contain in its more complex composition, with the corresponding advantages of manufacture, cost, storage, and use, the following leading features, *viz.*: gluey mucilaginous or gelatinous matter (which would include, as previously explained, gelatinous matter or other protein rendered fluid and non-jellified by the chlorid of calcium or other chlorids, etc., mentioned, and the other natural or artificial mucilaginous ingredients as just set forth in this paragraph), heat responsive, 85 sticky, resinous matter (which would include the rosin or other pitchy waxy resin and combinations and like materials, already mentioned, rendered fluid or semifluid with creosote, naphthalene, pure tar, or other 90 slow-drying, fluxing solvents and softeners), cheap, bulk-giving cementitious matter such as the starches and gums (as just mentioned in this paragraph) viscous oil (such as boiled linseed oil for increasing the 95 water repellent feature), fluxing matter such as the olein oil for also giving flexibility and a better union between the water fluxing mucilaginous component and the 100 sticky water-repellent heat-responsive component (although not requiring heat necessarily in use), glycerin (for softening and aiding the union of the water dissolved mucilaginous matter with the otherwise 105 opposing elements), a sticky gummy matter in naphtha solution (and preferably containing both rubber and gutta-percha-like substances) and body material such as cork in small chunks. In the foregoing filler, 110 where the toughening component is diffused through a large mass of binding material it becomes a tough tempering medium after the filler has set, and when very plastic, or smooth-flowing, a little of it (along with the other sticky cementing materials) may 115 be spread throughout a large mass of the bulk-forming and body materials. The chlorid renders the glue (or like element) mucilaginous and fluid, instead of jellified (when cold) but is not a softening solvent, 120 and the soluble oils and glycerin act on both the mucilaginous matter (*i. e.* the water responsive matter) and the gummy, sticky, cementitious matter (*i. e.* the heat responsive, water repellent matter or elements) and renders them softer and less brittle when set (which condition the chlorid could not maintain at this stage of the use of the filler). The slow drying property 125 is due to the dissolving influence of the 130

chlorid in the first instance, and then to the naphthalene and other non-aqueous solvents mentioned and to the olein. The viscous oil and gums mentioned are capable, in this combination, of an extremely fine dissemination and therefore more capable of spreading the water repellent influence throughout the mass in a way which materially improves the quick setting, slow-drying feature, which is the paramount feature aimed at. The volatile fluidifying agent or agents, whether primarily water or naphtha, aids this same feature, and the use of both in the combination, as explained, facilitates the combination of (together with the advantages of) the glue, which is responsive to water, but not to naphtha, and the other gums, etc., which are readily soluble in naphtha, and not in water.

My invention also includes combinations of ingredients which do not flux in the same sense as the first specific formula mentioned, but which, on account of the thick fluidity of the preparation, permit the opposing sticky ingredient to dissolve better so as to spread throughout the mass in a finer solution, finer dissemination or subdivision and state of more nearly complete fluidity or molecular separation, so that its sticky nature becomes sufficiently active and uniform among the granules of the cork mass to fulfil the desired purpose for a shoe-bottom filler. The species of this combination forms the subject matter of my divisional application, Serial No. 707,745, filed July 5, 1912, which is in part a continuation of and largely divided from my application, Serial No. 432,083, filed May 11, 1908 (and since become Pat. No. 1,032,812), where the same is broadly claimed, the invention therein disclosed including this form of my present invention, excepting that it does not include the slow-drying feature of the gluey component. For instance, I find this to be the case with petroleum wax tailings, used in connection with the glue-portion of the filler preparation above described. The reason for this is that the saponifying influence which is possible with resins cannot be developed on these petroleum pitches, and hence it is only in a heated state that I am able to secure the homogeneous conditions required in the cement liquid, which, upon cooling, shows the required finely divided separation and distribution of the mineral pitch. While, therefore, the preferable perfect chemical subdivision or union of the ingredients in the formulas previously discussed is lacking in the compound now being explained, this objection is not noticeable in the set granulated filler mass, and accordingly, because of the extremely sticky nature of this compound and also from a standpoint of economy, it is sometimes preferable, or, if not wholly so, it is

at times desirable to substitute the mineral pitch, at least in part, for the rosin or the like in the preceding formulas.

Adverting now again to the tenacity-giving member of my preparation, namely the glue, it is to be noted that the glue, gelatin, or like materials, possess great binding qualities, especially noticeable with granulated cork. This latter material, when slightly coated with my gluey binder, forms in itself a fairly resilient mass, the resiliency of the granulated cork mass being greatly improved by overcoming the normal brittle nature of the glue, as explained, either with glycerin or with olein oil or both or with combinations of thick viscous bodies, as explained. While glue, properly so called, is preferred for the reasons already stated, I include among the gluey constituents of my binding agent or preparation, considered as a whole, casein, flour, starch, dextrins (or artificial gums made from starch), natural gums such as gum arabic, etc., but I do not intend to depend entirely for the tenacious quality upon solutions containing these starchy or gummy solutions, but I select sticky, resinous ingredients having a permanent toughness (such as the resinous vegetable gums mentioned in said patent) or impart (by means of viscous oils, for example, as stated in said patent) to the sticky resinous ingredients a permanent toughness, as has been already apparent and combine the same with the above firm-setting gluey constituents (such as the casein, flour, etc., just mentioned), so that the eventual union of the various ingredients will be sufficiently tough and firm as required for the shoe-bottom filler. When dextrin, casein, or starchy ingredients are used for the water-absorbing component or member, I prefer to supply to these ingredients softening means, such as olein oil or glycerin, or chlorid of zinc, or other chemical means for preventing the hardening of the cement coating of the granules, aside from or in addition to the fact that I supply to the sticky gummy resinous ingredients a permanent fluxing or softening agent (preferably oils or soft tarry liquids). This enables me to provide pliability and yielding qualities, derived from both the water repellent and water absorbent ingredients. Hence the resulting filler-mass remains conformable even after setting, and also retains proper tackiness for the desired purpose and length of time. For instance, one and one half parts of corn starch, nine parts of water, one half part of caustic soda (with a proper neutralizing quota of sulfuric acid), one and one half parts of alizarin oil, three parts rosin, one quarter part naphthalene, and one and one half parts vaseline, produces the desired filler binding agent. Another illustrative example for

rendering this feature of my invention more clearly understood is three parts of gum arabic, two parts glycerin, one part chlorid of calcium, four parts of the naphthalene 5 treated rosin (which is elsewhere referred to as a naphthalate, as already explained), and sufficient water to give the desired fluidity.

As I have explained fully the use of shoe-bottom fillers, whether used hot or cold, in my preceding patents, and as said use is also well known in the art, it is sufficient to say that, having prepared the liquid binding agent, it is intermixed with the cork in 10 the proportion of about one gallon of the liquid to four to five gallons of the granulated cork, so as to thoroughly and entirely coat each granule and bind all the granules together with the very thinnest possible 15 union of binding agent, sufficient merely to maintain the mass properly together as a homogeneous body. The filler thus made is readily laid or smoothed down into the shoe bottom by a usual spreading tool, simply 20 moistened.

This application contains the generic or foundation claims to cover broadly the quick-setting but slow-drying, sticky, resili- 25 ent fillers of a large number of species, together with specific claims limited to the species containing resinous ingredients made sticky by suitable agents. Many of the species disclosed in other copending cases, 30 (as, some of those in my Patents 1,032,312, dated July 9, 1912 and 1,121,689, dated December 22, 1914) are capable of such variation or slight change as to carry out my present invention, although the particular refinement or feature which I have em- 35 phasized above as constituting the broad invention herein is not elsewhere set forth. I refer to the said copending applications to emphasize the wide scope of the present invention.

Having described my invention, what I claim as new and desire to secure by Letters Patent is:

1. A shoe bottom filler, consisting of a permanently pliable and resili- 50 ent filler mass which is quicksetting to a non-flowing, strongly adhesive and cohesive condition and thereafter continues slow drying, as described, and containing comminuted filler material, substantially as described.

2. A shoe bottom filler, consisting of a 55 filler mass which is quick setting to a non-flowing, strongly adhesive and cohesive and moldable condition, and thereafter continues slow-drying and resili- 60 ent, said filler mass comprising comminuted filler material, united by a binder, consisting at least in part of glue in a mucilaginous condition, and a sticky, tenacious, water repellent component, substantially as described.

3. A shoe bottom filler, consisting of a

filler mass which is quick setting to a non-flowing, strongly adhesive and cohesive but moldable condition, and thereafter continues slow drying and resili- 70 ent, and comprising comminuted filler material and a binder, 75 said binder consisting at least in part of a glue in a mucilaginous condition, and a sticky, tenacious, water repellent component in proportions to render the mass water- 80 proof, substantially as described. 75

4. A shoe bottom filler, containing com- 85 minuted filler material admixed with a gelatinous body combined with a chemically coalescing or modifying means rendering the mixture slow drying and sticky, sub- 80 stantially as described.

5. A shoe bottom filler, containing com- 85 minuted filler material admixed with a gelatinous body combined with a chemically coalescing or modifying means and resinous matter, rendering the mixture slow drying 90 and sticky, substantially as described.

6. A shoe bottom filler, consisting of a quicksetting, gelatinous body mixed with 90 comminuted filler material and combined with chemically coalescing or modifying means, rendering the mixture slow drying 95 and sticky, substantially as described.

7. A shoe bottom filler, consisting of a quick setting, gelatinous body mixed with 95 comminuted filler material and combined with means, rendering the mixture slow drying and sticky, and having a permanent elasticity and resiliency, substantially as de- 100 scribed.

8. The herein described binder for shoe bottom filler, comprising a quick setting, gelatinous slow drying mass combined with low melting, slow drying, sticky, resinous ingredients, substantially as described.

9. A shoe bottom filler, comprising a quick setting, gelatinous slow drying mass combined with low melting, slow drying, sticky, resinous ingredients, and comminuted 105 filler material, substantially as described.

10. A shoe bottom filler, comprising a gelatinous mass chemically rendered slow 110 drying and sticky, combined with low melting, slow drying, sticky ingredients and comminuted filler material, substantially as 115 described.

11. A shoe bottom filler, comprising a gelatinous mass chemically rendered slow 120 drying and sticky, combined with low melting, slow drying, sticky, waterproof in- 125 gredients and comminuted filler material, substantially as described.

12. A shoe bottom filler, comprising a gelatinous mass mixed with comminuted 125 filler material and having permanent elas- ticity and resiliency, chemically rendered slow drying and sticky, combined with low melting, slow drying, sticky components, substantially as described.

13. A shoe bottom filler, comprising a 130

- 8
6. A gelatinous binding agent, combined with chemically disintegrating and softening means rendering the cementitious mass quick setting, sticky and permanently flexible, admixed with body-giving comminuted filler material, substantially as described.
14. A shoe bottom filler, comprising a quick setting, sticky, flexible, gelatinous binding agent, combined with a low melting, sticky, resinous slow drying component, and admixed with a body-giving comminuted filler material, substantially as described.
10. A shoe bottom filler, comprising a quick-setting, sticky, flexible, elastic gelatinous binding agent combined with a water repellent, low melting slow drying mass and a body-giving filler material, substantially as described.
15. A shoe bottom filler, comprising a quick setting, sticky, flexible, elastic gelatinous binding agent combined with a water repellent, fluxing means rendering the cementitious mass water repellent and slow drying, and a body-giving filler material, substantially as described.
16. A shoe bottom filler, comprising a quick setting, sticky, flexible, elastic gelatinous binding agent, combined with water repellent, fluxing means rendering the cementitious mass water repellent and slow drying, and a body-giving filler material, substantially as described.
20. A shoe bottom filler, comprising a mucilaginous binding agent, combined with sticky flexible adhesive water-repellent ingredients and comminuted filler material in a mass slow-drying and water-repellent, substantially as described.
25. A shoe bottom filler, comprising a water-repellent resinous sticky component, containing the described product of rosin and naphthalene, combined with a gelatinous binding agent treated with chlorid of calcium, and admixed with comminuted filler material, substantially as described.
30. A shoe bottom filler binder, comprising a water repellent, resinous, sticky, component, combined with a gelatinous binding agent treated with a water soluble oil for facilitating said combination or fluxing, substantially as described.
35. A shoe bottom filler, comprising an elastic and flexible gelatinous mass combined with olein oil and incorporated with water repellent ingredients to render the mass waterproof, permanently elastic and resilient, and admixed with granulated filler material to a semi-solid, self-sustaining consistency, substantially as described.
40. A shoe bottom filler, comprising gelatinous matter in combination with glycerin and olein oil for rendering the mass flexible and elastic, and water repellent, resinous, tarry, oily ingredients, admixed with comminuted filler material, substantially as described.
45. A shoe bottom filler, comprising a water soluble mucilaginous component and a resinous ingredient in solution with water soluble oil, and admixed with body material to a plastic moldable consistency elastic when set, substantially as described.
50. A shoe bottom filler, comprising a gluey component rendered fluid and slow drying by a dissolving agent and admixed with body material to a plastic condition permanently pliable and resilient when set, substantially as described.
55. A shoe bottom filler, comprising a gluey component in solution with chlorid of calcium, and admixed with body material, substantially as described.
60. A shoe bottom filler, consisting of a water soluble proteid in solution with water soluble oil, united with sticky adhesive waterproof material and admixed with body material, substantially as described.
65. A shoe bottom filler, consisting of a water soluble proteid in solution with water soluble oil, united with sticky, adhesive waterproof material, and admixed with comminuted filler material to a self-sustaining consistency, substantially as described.
70. A shoe bottom filler component, consisting of a water soluble proteid in solution with water soluble oil, united with sticky, resinous materials but having the water solvent substantially evaporated to render the same capable of subsequent solution in naphtha, substantially as described.
75. A shoe bottom filler component, consisting of soluble, gelatinous matter in solution with a water-soluble oil admixed with sticky, adhesive, water repellent ingredients in solution, substantially as described.
80. A shoe bottom filler, consisting of comminuted filler material admixed with a compound consisting of a binding agent containing proteid and starch in proportions to render the combination sticky and adhesive, and a water repellent, resinous component, substantially as described.
85. A shoe bottom filler, consisting of a quick setting, gelatinous and starchy mass combined with low melting, slow drying, sticky, resinous ingredients, and comminuted filler material, substantially as described.
90. A shoe bottom filler, consisting of a quick setting, gelatinous and starchy mass combined with low melting, slow drying, sticky, resinous ingredients in proportion to make the mass water repellent, elastic and resilient, and comminuted filler material, substantially as described.
95. A shoe bottom filler, consisting of a quick setting, gelatinous and starchy mass combined with low melting, slow drying, sticky, resinous ingredients, and comminuted filler material, substantially as described.
100. A shoe bottom filler, consisting of a quick setting, gelatinous and starchy mass combined with low melting, slow drying, sticky, resinous ingredients, and comminuted filler material, substantially as described.
105. A shoe bottom filler, consisting of a quick setting, gelatinous and starchy mass combined with low melting, slow drying, sticky, resinous ingredients, and comminuted filler material, substantially as described.
110. A shoe bottom filler, consisting of a quick setting, gelatinous and starchy mass combined with low melting, slow drying, sticky, resinous ingredients, and comminuted filler material, substantially as described.
115. A shoe bottom filler, consisting of a quick setting, gelatinous and starchy mass combined with chemically disintegrating and softening means, and sticky resinous matter rendering the cementitious mass quick setting, sticky and flexible, admixed with comminuted filler material, substantially as described.
120. A shoe bottom filler, consisting of a gelatinous and starchy mucilaginous binding agent combined with chemically disintegrating and softening means, and sticky resinous matter rendering the cementitious mass quick setting, sticky and flexible, admixed with comminuted filler material, substantially as described.
125. A shoe bottom filler, which is quick setting and slow drying comprising a mucilaginous binding agent combined with sticky, flexible, adhesive, water repellent ingredients and comminuted filler material in

a mass permanently pliable and resilient, substantially as described.

34. A shoe bottom filler, consisting of a binding agent composed of gelatinous matter in a solution containing olein oil and naphthalene compounded with rosin, admixed with comminuted filler material, substantially as described.

35. A shoe bottom filler, consisting of starch jellified to a highly expanded state as by alkali, combined with a chemically coalescing or modifying means rendering the mixture quicksetting and slow drying, admixed with comminuted filler materials, substantially as described.

36. A shoe bottom filler, consisting of starch jellified to a highly expanded state as by the chemical action of alkalis and acids, combined with a chemically coalescing or modifying means rendering the mixture quicksetting and slow drying, admixed with comminuted filler material to a semi-solid, self-sustaining consistency, substantially as described.

37. A shoe bottom filler, which is quick setting and slow drying, comprising gelatinized matter in solution with olein oil, combined with adhesive ingredients and comminuted filler material, in a permanently tough and adhesive mass, substantially as described.

38. A shoe bottom filler, which is quick setting and slow drying, comprising comminuted filler material admixed with gelatinous matter in solution with olein oil, combined with slow drying, sticky ingredients rendering the mixed mass plastic and conformable to the extent required for the practical laying of shoe bottoms, substantially as described.

39. A shoe bottom filler, which is quick setting and slow drying, comprising glue in solution with olein oil, fluxed with water repellent, sticky matter, in which the water portions of the oil are sufficiently evaporated to permit the thinning of the preparation by naphtha, combined with said naphtha, and admixed with comminuted filler material, substantially as described.

40. A shoe bottom filler, which is quick setting and slow drying, comprising a gelatinous binding agent rendered soft and elastic by a chemical solvent rendered sticky and adhesive with resinous matter and creosote and comminuted filler material, substantially as described.

41. A shoe bottom filler, which is quick setting and slow drying, comprising comminuted filler material admixed with a normally fluid, gelatinous binding agent combined with tar-treated resinous ingredients rendering the preparation sticky, adhesive and conformable for sole laying purposes, substantially as described.

42. A shoe bottom filler, which is quick

setting and slow drying, comprising comminuted filler material, a gelatinous body rendered normally fluid by chlorid of calcium, and saponified, sticky, resinous ingredients, mixed together in an adhesive, elastic, permanently resilient mass, substantially as described.

43. A shoe bottom filler, which is quick setting and slow drying, comprising chemically treated gelatinous matter in a normally fluid condition, and emulsified, oily and resinous ingredients, admixed with ground cork into a sticky, flexible mass conformable to the sole-laying process when applied to the shoe bottoms, substantially as described.

44. A shoe bottom filler binder, permanently resilient, adhesive and elastic, comprising a gelatinous body rendered normally fluid by chlorid of calcium, and saponified, sticky, resinous ingredients, substantially as described.

45. A shoe bottom filler, consisting of a filler mass, which is quick setting to a strongly adhesive, cohesive, moldable condition, and thereafter continuous slow drying and permanently pliable, said filler mass consisting of comminuted filler material, mixed with a binder, comprising a water absorbent, gluey component, suitable chemical means for preventing hardening of said component, and sticky, resinous material, including rosin and naphthalene, substantially as described.

46. A shoe bottom filler, consisting of a filler mass, which is quick setting to a strongly adhesive, cohesive, moldable condition, and thereafter continues slow drying and permanently pliable, said filler mass consisting of comminuted filler material, mixed with a binder, comprising a water absorbent, gluey component, consisting at least in part of starch, chlorid of calcium, and sticky, resinous material, including rosin and naphthalene, substantially as described.

47. A shoe bottom filler, consisting of a filler mass which is quick setting to a strongly adhesive and cohesive, moldable condition, and thereafter continues slow drying and permanently pliable, consisting of comminuted filler material mixed with a binder, comprising a gelatinous body in a mucilaginous condition, and sticky resinous matter, consisting at least in part of viscous oil, and rosin, substantially as described.

48. A shoe bottom filler, consisting of a filler mass which is quick setting to a strongly adhesive and cohesive, moldable condition, and thereafter continues slow drying and permanently pliable, consisting of comminuted filler material mixed with a binder comprising a gelatinous body in a mucilaginous condition, and sticky resinous matter, consisting at least in part of viscous

- oil, rosin and naphthalene, substantially as described.
49. A shoe bottom filler, consisting of a filler mass which is quick setting to a strongly adhesive and cohesive, moldable condition, and thereafter continues slow drying and permanently pliable, consisting of comminuted filler material mixed with a binder comprising a gelatinous body in a mucilaginous condition, and sticky resinous matter, consisting at least in part of viscous oil, rosin, and a fluidifying agent rendering the mass moldable hot or cold, substantially as described.
50. A shoe bottom filler, consisting of a filler mass which is quick setting to a strongly adhesive and cohesive, moldable condition, and thereafter continues slow drying and permanently pliable, sticky and tough, comprising comminuted filler material mixed with a binder, comprising gelatinous material, rendered slow drying with chlorid of calcium, and sticky resinous material, containing rosin combined with naphthalene, said mass being in a condition moldable hot or cold, substantially as described.
51. A shoe bottom filler, consisting of a filler mass which is quick setting to a strongly adhesive and cohesive, moldable condition, and thereafter continues slow drying and permanently pliable, sticky and tough, comprising comminuted filler material, mixed with a binder, comprising mucilaginous matter, rendered slow drying with chlorid of calcium, and permanently pliable with glycerin, and sticky resinous material, containing rosin and naphthalene, substantially as described.
52. A shoe bottom filler, consisting of a filler mass which is quick setting to a strongly adhesive and cohesive, moldable condition, and thereafter continues slow drying and permanently pliable, sticky and tough, comprising comminuted filler material mixed with a binder, comprising gelatinous material, rendered slow drying with chlorid of calcium, and permanently pliable with glycerin, and sticky resinous material, containing rosin and naphthalene, said mass having the union of its gelatinous and resinous materials promoted with olein oil, substantially as described.
53. A shoe bottom filler, consisting of a filler mass which is quick setting to a strongly adhesive and cohesive and moldable condition, and thereafter continues slow drying and permanently pliable, consisting of comminuted filler material mixed with a binder comprising gelatinous matter treated with glycerin and olein oil, and united in a naphtha solution with a naphtha soluble sticky gum, substantially as described.
54. A shoe bottom filler, consisting of a filler mass which is quick setting to a strongly adhesive, and cohesive, moldable condition, and thereafter continues slow drying and permanently pliable, consisting of comminuted filler material mixed with a binder comprising gelatinous matter treated with glycerin and olein oil, and united in a naphtha solution with a naphtha soluble sticky gum, consisting at least in part of rubber-like materials, substantially as described.
55. A shoe bottom filler, consisting of a filler mass which is quick setting to a strongly adhesive, and cohesive, moldable condition, and thereafter continues slow drying and permanently pliable, consisting of comminuted filler material mixed with a binder comprising gelatinous matter treated with glycerin and olein oil, and united in a naphtha solution with a naphtha soluble sticky gum, consisting at least in part of rubber-like material, (including the gutta-perchas and pseudo-gutta-perchas in this term), substantially as described.
56. In a shoe bottom filler, a light weight, fibrous body material, mixed with a pasty ingredient and an oily softener to a permanently pliable, tough consistency adapted to a shoe bottom.
57. In a shoe bottom filler, a comminuted body material, mixed with a pasty ingredient and an oily softener, including a water-soluble oil and having a slow-drying characteristic.
58. A shoe bottom filler, comprising a body material, mixed to a tough, sticky, flexible, self-sustaining consistency with a compound including a gluey gum, and a naphtha solution of a paste-making ingredient.
59. A shoe bottom filler, comprising a comminuted body material, mixed to a tough, sticky, flexible, sustaining consistency with a compound including a resinous ingredient and a paste-making ingredient, united in a naphtha solution.
60. A shoe bottom filler, comprising a comminuted body material, mixed with a compound including the described product of resin and naphthalene and a paste-making ingredient.
61. A shoe filler, containing fragmentary body material united by a binding agent comprising a paste making ingredient in a permanently jellified condition and softened and rendered tenacious by a water-soluble fat-derived oil.
62. A shoe filler, containing fragmentary body material united by a binding agent comprising a permanently jellified, starchy ingredient chemically softened and rendered tenacious.
63. A shoe filler, comprising a fragmentary body material united by a binding

agent containing a jellified adhesive softened and rendered tenacious by an oil.

64. A shoe filler, comprising a fragmentary body material united by a binding agent containing a naphtha solution of a so-called rubber gum.

In testimony whereof, I have signed my

name to this specification, in the presence of two subscribing witnesses.

Witnesses: ANDREW THOMA.

M. J. SPALDING,  
EDWARD MAXWELL.

It is hereby certified that in Letters Patent No. 1,134,931, granted April 6, 1915, upon the application of Andrew Thoma, of Cambridge, Massachusetts, for an improvement in "Shoe-Bottom Fillers," errors appear in the printed specification requiring correction as follows: Page 7, line 101, after the word "for" insert the article *a*; page 8, lines 76, 81, 87, 94, 99, 106, 111, and 118, for the words "consisting of" read *comprising*; page 9 lines 3, 9, and 16, for the words "consisting of" read *comprising*; same page, line 91, for the word "continuous" read *continues*; page 10, line 105, for the word "sustaining" read *self-sustaining*; and that the said Letters Patent should be read with these corrections therein that the same may conform to the record of the case in the Patent Office.

Signed and sealed this 18th day of May, A. D., 1915.

[SEAL.]

R. F. WHITEHEAD,  
*Acting Commissioner of Patents.*